

## UNITED STATES PATENT OFFICE.

LUTHER P. BROWN, OF NORTH ADAMS, MASSACHUSETTS.

## COMPOSITION FOR WATERPROOFING.

SPECIFICATION forming part of Letters Patent No. 793,048, dated June 27, 1905.

Application filed November 6, 1903. Serial No. 180,078.

*To all whom it may concern:*

Be it known that I, LUTHER P. BROWN, a citizen of the United States, residing at North Adams, in the county of Berkshire and State 5 of Massachusetts, have invented a new and useful Composition for Waterproofing Cartons or Receptacles, of which the following is a specification.

This invention is a composition for rendering paper cartons or receptacles water and liquid proof.

The object of the invention is to provide a composition which when applied to a paper or pulp carton or receptacle will impregnate and 15 coat the same, so as to render the said carton or receptacle capable of holding any and all liquids and materials containing liquids or ingredients which ordinarily soak through and escape from an ordinary paper receptacle 20 or package.

With this object in view the invention consists in the ingredients combined in a manner hereinafter fully described, and pointed out in the claim.

25 In compounding the composition which constitutes my invention I employ paraffin-wax, paraffin-oil, Brazilian wax, talc, asbestos, asbestine, powdered chalk, beeswax, bayberry-wax, petroleum-oil, ceresin-wax, and white 30 wax. These ingredients are used in the following proportions: eight parts paraffin-wax, one part paraffin-oil, three parts Brazilian wax, six parts talc, two parts asbestos, four parts asbestine, one part powdered chalk, one part 35 beeswax, one part bayberry-wax, one part petroleum-oil, one part ceresin-wax, and one

part white wax. These ingredients are placed in a suitable receptacle and heated until the entire mass becomes a homogeneous liquefied composition, and the paper receptacle or carton is immersed in the said composition while heated at its liquefied temperature and is permitted to remain therein a sufficient length of time to become thoroughly impregnated and coated upon the interior and exterior with 45 the said composition.

It will be understood that the ingredients embrace three distinct classes of materials—namely, wax, oils, and earthy or calcareous material—combined with asbestos or some 50 material formed from asbestos. The materials mentioned, however, and in the proportion specified I believe to be the best adapted for carrying out the purpose of my invention. It will also be understood that this 55 composition can be used for waterproofing paper in flat sheets, so that said paper can be used for wrapping or manufacturing purposes.

Having thus fully described my invention, what I claim as new, and desire to secure by 60 Letters Patent, is—

A composition for rendering paper cartons or receptacles liquid-proof and consisting of paraffin-wax and paraffin-oil, Brazilian wax, talc, powdered asbestos, asbestine, powdered 65 chalk, beeswax, bayberry-wax, petroleum-oil, ceresin-wax and white wax in the proportions specified.

LUTHER P. BROWN.

Witnesses:

LILLIAN V. BRADFORD,  
LOUIS C. CHASE.